

Feb. 16, 1926.

1,573,784

J. W. VAN METER

PROCESS OF TEMPERING METALS AND OTHER MATERIALS

Filed June 9, 1922

*Fig. 1.*



*Fig. 2.* *Fig. 3.*



Inventor

James W. Van Meter

21 By

J. W. Garner

Attorney

Patented Feb. 16, 1926.

1,573,784

# UNITED STATES PATENT OFFICE.

JAMES W. VAN METER, OF SAN RAFAEL, CALIFORNIA.

## PROCESS OF TEMPERING METALS AND OTHER MATERIALS.

Application filed June 9, 1922. Serial No. 567,096.

To all whom it may concern:

Be it known that I, JAMES W. VAN METER, a citizen of the United States, and resident of San Rafael, in the county of Marin, 5 State of California, have invented a new and useful Process of Tempering Metals and Other Materials, of which the following is a specification.

This invention relates to improvements in 10 methods of tempering and case hardening steel and other material by the use of cyanides, such as sodium, potassium, and alkaline cyanides, the object of the invention being to provide an improved method by 15 which steel or other material can be tempered in a very short time, at minimum cost, without the employment of expensive furnaces or apparatus, or of fire or electric current, and without danger of poisoning 20 the operative, and consists in exposing such material to the action of gases generated by the chemical reaction of a reaction causing agent, for instance, chlorine, on a body of initially inert material for instance, particles of zinc, iron, lead, arsenic, or other metal, and on salts of cyanide, especially sodium cyanide, and potassium cyanide, as 25 hereinafter described and claimed.

In the accompanying drawing:—

30 Fig. 1 is a diagram, partly in elevation, and partly in section, showing an internal combustion engine cylinder, arranged to be tempered on the inside, in accordance with my improved tempering method.

35 Fig. 2 is a similar view, showing a body of metal in the act of being tempered on the exterior in accordance with my improved method.

40 Fig. 3 is a similar view, showing a plow plate being tempered on only one exterior surface in accordance with my method.

45 My improved method is especially adapted for tempering hollow bodies such as internal combustion engine cylinders on the inside, and for tempering metallic articles, such as for instance plow plates, moldboards, dies and the like on the working side, from the exterior, but may also be used for tempering an article or body of metal or other material throughout its entire extent.

50 In carrying out my improved method, I provide a sufficient charge or body of inert material which may consist preferably of sawdust, which contains some moisture, 55 bran or the like, and mix the same intimately with an initially inert material,

such as for instance particles of iron, lead, zinc, arsenic, or other metal, and also with salts of cyanide, such as sodium cyanide, or potassium cyanide, or cyanides of the alkaline earths, and also preferably with benzol or hydrocarbon oil to act as a binder and also as a combustible agent.

Such material is generally used in about 60 the following proportions:—

Sawdust, 1 pound; iron filings, 2 pounds; sodium cyanide,  $\frac{1}{2}$  pound; benzol or hydrocarbon oil,  $\frac{1}{2}$  pound.

Assuming that the article to be tempered is the cylinder 1 of an internal combustion engine, and that the same is to be tempered on the inside, to render the same exceedingly hard on its inner surface and thereby minimize wear or enlargement of the cylinder bore by the piston, I fill such cylinder with 70 a charge of such material, as indicated at 2, secure the head 2<sup>a</sup> on the cylinder, close the valve opening with a plug 2<sup>b</sup>, and close the lower end of the cylinder with a suitable closure 3, which is here shown as securely 75 held in place by means of hook bolts 4. An escape pipe 5 leads from the closure to the outer air at a suitable point or to a suitable vessel of water or other place where the fumes may be absorbed or neutralized, and 80 this pipe is provided with a valve 6 to enable said pipe to be opened or closed to any desired extent or at any time required as may be necessary to enable any desired pressure to be attained in the cylinder while 85 the same is being tempered.

I also provide a suitable quantity of a reaction causing agent, such as for instance, chlorine, which is here shown diagrammatically as contained under pressure in a liquid 95 state in a tank 7. Said tank has a valve 8 which may be opened or closed at will to control the passage of chlorine gas from the tank to the cylinder or other work through a tube 9 which is here shown as entering the 100 cylinder through a suitable stopper 10 which is placed in the opening from which the spark plug was removed. I also provide means to force air through the said tube to the charge or body of inert material in the 105 cylinder or other work, and for this purpose I here show a container 11 for compressed air, which container is provided with a suitable controlling valve 12 and communicates with the tube 9 through a tube 13.

I first keep the valves 6 and 12 closed and open the valve 8 to liberate chlorine gas

which then passes through the pipe 9 to the charge 2 in the engine cylinder. The chemical reaction of the chlorine on the metallic particles causes intense heat to be instantly developed, without the aid of oxygen, and to which the interior of the cylinder is exposed, and at the same time such heat brings about the dissociation of the sodium cyanide, thereby causing cyanogen to be liberated.

- 10 Leaving the valve 6 closed, the valve 8 may be also closed when a sufficient quantity of the chlorine has been used and the valve 12 opened to cause compressed air to also enter the cylinder and by appropriately 15 manipulating the valve 12 the compressed air may be used to a sufficient extent to regulate the temperature in the cylinder, to give the required degree of hardness or temper to the inner surface of the cylinder.
- 20 When the tempering has been effected the valve 6 is then opened and compressed air employed to scavenge the cylinder and drive out the poisonous fumes which are conveyed through the pipe 5 to a suitable 25 point, and are hence rendered innocuous, and danger to the operative is avoided.

Pressure and heat on the cyanide make it extremely effective in tempering the work. Moreover, my improved method enables a 30 material economy of cyanide to be effected as a comparatively small quantity of the cyanide is all that is required by my improved method for tempering a surface of considerable area. All the cyanide is confined and liberated in the cylinder under 35 pressure, and hence its tempering effect is much more rapid than when it is used in the open by the process heretofore employed, and moreover there is a certain amount of 40 case hardening or carburizing action.

Another advantage resulting from the use of my improved process is that the interior surface of the work can be instantaneously heated to the required degree for tempering 45 such surface, and without heating the body of the work throughout, when this is desired, and thus the tempering is confined to the wearing surface, without being appreciably imparted to the remainder of the body of 50 the work. When the work is thus tempered only on one surface, the untempered portion of the body acts as a cushion behind such tempered surface or portion.

My improved method can also with equal 55 facility be employed for tempering an object from the outside. In Fig. 2, I show a furnace 14 in which the work 15 is embedded in a charge 16 of the initially inert material, the chlorine being introduced through a pipe 17, and the gases emitted through a flue 18.

When it is desired to temper only one 60 exterior surface of a metallic object, such as for instance, a plow iron, the work 19, shown in Fig. 3, is arranged with only one

surface in contact with the charge 20 of the initially inert material, the other surfaces of the work being protected by a bed 21 of suitable material such as for instance a paste composed of powdered asbestos mixed with 70 a sufficient quantity of saturated solution of sal ammoniac to render the same plastic.

While I have herein described a specific mode of carrying out my improved process, I would have it understood that modifications may be made within the scope of my invention as defined in the appended claims.

In the preparation of the charge to be acted upon by the chlorine, I have used salts of cyanide, and have also used cyanides of the alkaline earths. I may omit both of them from the charge, and supply cyanogen or other tempering agent from an independent source to the work, while the work is in the heated condition resulting from its 35 exposure to the heat generated by the chemical reaction of the chlorine or other reaction causing agent, on the metallic particles, or other initially inert material, and I do not limit myself in such particulars. 90

I claim:—

1. Method of tempering consisting in heating the work in a non-oxidizing atmosphere and subjecting the same to the action of cyanogen. 95
2. Method of tempering, consisting in heating the work in a non-oxidizing atmosphere and subjecting the same to the action of cyanogen under pressure. 100
3. Method of tempering, consisting in heating the work in a non-oxidizing atmosphere, excluding the same from the outer air, and subjecting the same to the action of cyanogen. 105
4. Method of tempering, consisting in heating the work in a non-oxidizing atmosphere, excluding the same from the outer air, and subjecting the same to the action of cyanogen under pressure. 110
5. Method of tempering, consisting in exposing the work to heat generated by the chemical reaction of a reaction causing agent, on initially inert material, in the presence of salts of cyanide. 115
6. Method of tempering, consisting in exposing the work to heat generated by the chemical reaction of a reaction causing agent on initially inert material in a non-oxidizing atmosphere in the presence of salts of cyanide, and regulating the temperature of the work during the tempering thereof. 120
7. Method of tempering, consisting in excluding the work from the outer air, and exposing the work to heat generated by the chemical reaction of a reaction causing agent on initially inert material in a non-oxidizing atmosphere in the presence of salts of cyanide. 125
8. Method of tempering, consisting in ex- 130

cluding the work from the outer air, and exposing the work to heat generated by the chemical reaction of a reaction causing agent on initially inert material in a non-  
5 oxidizing atmosphere in the presence of salts of cyanide and under pressure.

9. Method of tempering, consisting in exposing the work to heat generated by the chemical reaction of a reaction causing  
10 agent on initially inert material in a non-  
oxidizing atmosphere in the presence of salts of cyanide and under pressure.

10. Method of tempering a hollow body, consisting in exposing the interior thereof  
15 to heat generated by the chemical reaction of a reaction causing agent on initially inert material in a non-oxidizing atmosphere in the presence of salts of cyanide.

11. Method of tempering a hollow body,  
20 consisting in exposing the interior thereof to heat generated by the chemical reaction of a reaction causing agent on initially inert material in a non-oxidizing atmosphere in the presence of salts of cyanide and under  
25 pressure.

12. Method of tempering a hollow body, consisting in exposing the interior thereof to heat generated by the chemical reaction of a reaction causing agent on initially  
30 inert material in a non-oxidizing atmosphere in the presence of salts of cyanide and under pressure and regulating the temperature of the heated interior surface by the application of a cooling medium thereto.

35 13. Method of tempering, consisting in exposing the work to heat generated by the chemical reaction of a reaction causing agent on initially inert material in a non-  
oxidizing atmosphere in the presence of salts  
40 of cyanide.

14. Method of tempering a surface of a body, consisting in exposing such surface to heat generated by the chemical reaction of a reaction causing agent on initially inert material in a non-oxidizing atmosphere in  
45 the presence of salts of cyanide, and protecting other surfaces of such body from such heat.

15. Method of tempering, consisting in exposing the work to heat generated by the  
50 chemical reaction of a reaction causing agent, on inert material, in the presence of an alkaline cyanide.

16. Method of tempering, consisting in exposing the work to heat generated by the  
55 chemical reaction of a reaction causing agent on initially inert material in a non-oxidizing atmosphere in the presence of an alkaline cyanide, and regulating the temperature of the work during the tempering  
60 thereof.

17. In the process of tempering, the step of heating the work to the required temperature for the action of the tempering agent, by exposing the work to the heat generated  
65 by the chemical reaction of a reaction causing agent on initially inert material in a non-oxidizing atmosphere.

18. The process of tempering, consisting in heating the work to the required temperature for the action of the tempering agent by exposing the work to the heat generated  
70 by the chemical reaction of a reaction causing agent on initially inert material in a non-oxidizing atmosphere. and applying  
75 such tempering agent to the heated work.

In witness whereof I affix my signature.

JAMES W. VAN METER.